# EUROPEAN PATENT SPECIFICATION

(11) **EP 0 551 702 B1**
(45) Date of publication and mention of the grant of the patent: **10.06.1998**
(21) Application number: 92302169.5
(22) Date of filing: 13.03.1992
(51) Int. Cl.: C23C 8/34

(54) **Method of nitriding nickel alloy**
Verfahren zum Nitrieren von einer Nickel-Legierung
Procédé de nitruration d'un alliage de nickel

(30) Priority: 14.01.1992 JP 24763/92
(43) Date of publication of application: 21.07.1993
(73) Proprietor: DAIDO HOXAN INC., Sapporo-city (JP)
(72) Inventor: Tahara, Masaaki, Takatsuki-shi, Osaka 569 (JP); Senbokuya, Haruo, Tondabayashi-shi, Osaka 584 (JP); Kitano, Kenzo, Kawachinagano-shi, Osaka 586 (JP); Hayashida, Tadashi, Sakai-shi, Osaka 593 (JP); Minato, Teruo, Hashimoto-shi, Wakayama 648 (JP)
(74) Representative: Marlow, Nicholas Simon

(56) References cited:
- EP-A- 0 352 061
- EP-A- 0 408 168
- US-A- 3 129 124
- PATENT ABSTRACTS OF JAPAN vol. 8, no. 98 (C-221)(1535) 9 May 1984

## Description

This invention relates to a method for nitriding nickel alloy for the improvement of surface hardness and other properties by forming a nitrided layer on nickel alloy surface.

Alloy with a high nickel content, such as as inconel(Ni-Cr), hastelloy(Ni-Cr-Mo) and incolloy,has been becoming widely employed because of its superior heat resistance and corrosion resistance. Recently there is an increasing demand for improving wear resistance and other properties of alloy containing nickel and expanding its applicable fields. However, for the above-mentioned nickel alloy such as inconel, the method for the improvement of surface hardness has not been established yet. A method of push-out hardening for the improvement of base material intensity and a use of superplastic articles employing powder material are merely studied. However, since the method of push-out hardening increases stiffness of whole alloy, workability of the alloy is damaged. Also superplastic articles employing powder material are difficult to put into practical use due to extremely high cost.

Conventional methods of surface hardening for general metallic materials are as follows, ① a plating method, ② a coating method such as PVD, and ③ a diffusion method such as nitriding and boriding. However, for nickel alloy, only some of the coating methods, such as full hard chrome plating and alumina coating, find practical use as mentioned above. Those methods have difficulty in quality control which is peculiar to the coating method, and limit the application range due to the thinness of the coating. Moreover, high cost for treatment is another problem. For the diffusion method of surface hardening, plasma ion nitriding using glow discharge has been also tried partly for inconel alloy and hastelloy alloy. However, the treatment of such plasma ion nitriding scarcely forms a hardened nitrided layer on the above-mentioned nickel alloy. Even if formed, that would be a partly formed ultra thin layer only several µm (microns) deep. Therefore, in the present situation, nitriding the above-mentioned nickel alloy is almost given up and far from turning it to practical use.

EP 0 408 168 discloses the pre-nitriding fluorination of stainless steel SUS 305, which contains 10.5-13.0% Ni, at a temperature of 350°C.

The present invention can provide a method of nitriding nickel alloy containing more than 25% nickel for the improvement of the surface hardness of nickel alloy by which a uniformly nitrided deep layer can be formed on the nickel alloy surface.

The present invention provides a method for nitriding nickel alloy which comprises steps of holding nickel alloy containing more than 25% nickel in a fluorine or fluoride-containing gas atmosphere withheating at a temperature of 550-600°C and holding the fluorinated nickel alloy in a nitriding atmosphere with heating to form the surface layer of the nickel alloy into a nitrided layer.

The method of the invention is applied to a nickel alloy, which is nitrided in a nitriding atmosphere after having been fluorided in a fluorine- or fluoride-containing gas atmosphere.

Nickel alloys containing more than 25 weight % (it will be abbreviated to " % " hereafter) nickel, for example, Ni-Cr, Ni-Cr-Mo, and Ni-Cr-Fe are used in the method of the invention. Examples of such alloys with a high nickel content are inconel, hastelloy, and incolloy.

A method does not specify a shape of nickel alloy nor a level of processing. All the material, intermediate products, and finished products made of nickel alloy are included to the extent of nickel alloy in this invention.

Fluorine- or fluoride-containing gas for a fluorine- or fluoride-containing gas atmosphere, in which the above-mentioned nickel alloy is reacted, is fluorine compound gas, such as NF₃, BF₃, CF₄, HF, SF₆, C₂F₆, WF₆, CHF₃, or SiF₄. They are used independently or in combination. Besides, fluorine compound gas with F in its molecule can be used as the above-mentioned fluorine- or fluoride-containing gas. Also F₂ gas formed by cracking fluorine compound gas in a heat decomposition device and preliminarily formed F₂ gas are employed as the above-mentioned fluorine- or fluoride-containing gas. According to the case, such fluorine compound gas and F₂ gas are mixed for use. The above-mentioned fluorine or fluoride-containing gas such as the fluorine compound gas and F₂ gas can be used independently, but generally are diluted by inert gas such as N₂ gas for the treatment. The concentration of the fluorine- or fluoride-containing gas itself in such diluted gas should amount to , for example, 10,000 to 100,000ppm, preferably 20,000 to 70,000ppm, more preferably 30,000 to 50,000ppm.

In the invention, the above-mentioned nickel alloy is held in a heated condition in a fluorine- or fluoride-containing gas atmosphere of such concentration, and fluorided. This is the most characteristic part of the invention. In this case, nickel alloy is held with heating at a temperature of 550-600°C. The holding time of the above-mentioned nickel alloy in a fluorine- or fluoride-containing gas atmosphere may appropriately be selected depending on the nickel alloy species, geometry and dimension of the alloy, heating temperature and the like, generally within the range of about ten minutes toseveral hours. 30 minutes is a preferred exposure time. The treatment of nickel alloy in such fluorine- or fluoride-containing gas atmosphere allows "N" atoms to penetrate into nickel alloy, which was impossible in the past.

Though the mechanism of the penetration has not yet been proven, it can be largely understood as follows.

The oxidized layer of NiO formed on the nickel alloy surface inhibits penetration of "N" atoms for nitridation. upon holding nickel alloy with an oxidized layer in a fluorine- or fluoride-containing gas atmosphere with heating as mentioned above, the oxidized layer of NiO is converted to a fluorinated layer of NiF₂. "N" atoms for nitridation penetrate more readily into the fluorinated layer of NiF₂ than into the oxidized layer of NiO, that is, a nickel alloy surface is formed which is in a suitable condition for the penetration of "N" atoms by the above-mentioned fluorination. Thus, it is considered that "N" atoms in the nitriding gas penetrate uniformly into nickel alloy to a certain depth when nickel alloy is held in a nitriding atmosphere with such a suitable surface condition to absorb "N" atoms as follows, resulting the formation of a deep uniform nitriding layer.

Then, as mentioned above, nickel alloy with suitable surface condition to absorb "N" atoms by fluorination is held with heating in a nitriding atmosphere to nitride. In this case, nitriding gas composing a nitriding atmosphere is a simple gas composed of NH₃ only, or a mixed gas composed of NH₃ and a carbon source gas, for example, RX gas. Mixture of both gases can be also used. Generally, the above-mentioned simple gas mixed with an inert gas such as N₂ is used. According to the case, H₂ gas is added to those gases.

In such a nitriding atmosphere, the above-mentioned fluorinated nickel alloy is held with heating. A heating condition is generally set at a temperature of 500 to 700°C, and treatment time is set within the range of 3 to 6 hours. By this nitriding treatment, a close nitriding layer (consisting of entirely single layer) is formed deeply and uniformly on the surface of the above-mentioned nickel alloy, whereby the surface hardness of nickel alloy reaches Hv=800 to 1100 in comparison with that of base material thereof Hv=280 to 380. Thickness of the hardened layer basically depends on the nitriding temperature and time. However the temperature below 500 °C causes difficulty in forming a nitriding layer, and at the temperature over 650 °C, a fluorinated layer is damaged and Ni is easily oxidized thereby resulting in a tendency of unevenly nitrided layer formation.

On the other hand, a sufficient fluorinated layer ordinarily can not be formed at the fluoriding temperature below 400 °C. Also the temperature over 600°C is not appropriate for an industrial process because furnace materials in a muffle furnace are worn out due to extreme fluoriding reaction. From a viewpoint of forming a nitriding layer, it is also preferable that the difference between fluoriding temperature and nitriding temperature is as small as possible. For example, a proper nitriding layer is not formed by nitriding given after fluoriding and cooling once.

The above-mentioned fluoriding and nitriding steps are, for example, taken in a metallic muffle furnace as shown in Fig. 1, that is, the fluoriding treatment is carried out first, and then nitriding treatment is put in practice at the inside of the muffle furnace. In Fig. 1, the reference numeral 1 is a muffle furnace, 2 an outer shell of the muffle furnace, 3 a heater, 4 an inner vessel, 5 a gas inlet pipe, 6 an exhaust pipe, 7 a motor, 8 a fan, 11 a metallic container, 13 a vacuum pump, 14 a noxious substance eliminator, 15 and 16 cylinders, 17 flow meters, and 18 a valve. Nickel alloy articles 10 are put in the furnace 1 and fluorided by introducing fluorine- or fluoride-containing gas atmosphere such as NF₃ with heating. The gas is lead into the exhaust pipe 6 by the action of vacuum pump 13 and detoxicated in the noxious substance eliminator 14 before being spouted out. And then, the cylinder 15 is connected with a duct to carry out nitriding by introducing nitriding gas into the furnace 1. After nitriding, the gas is spouted out via the exhaust pipe 6 and the noxious substance eliminator 14. Through the series of these operations, fluoriding and nitriding treatments are put in practice. Also a device in Fig. 2 can be employed instead of one in Fig. 1. This device comprises a fluoriding chamber on the left side and a nitriding chamber on the right side. In the figure, the reference numeral 2' are metallic containers, 3' a heater, 5' an exhaust gas pipe, 6' and 7' open-close covers, 11' a base, 21 a furnace body with adiabatic walls, and 22 a barrier movable up and down. The barrier 22 divides the inner space of the furnace body 21 into two chambers, 23 and 24. The chamber 23 is designed for a fluoriding chamber and 24 is for a nitriding chamber. The reference numeral 25 is a rack comprising two rails on which a metallic container 2' having nickel alloy articles therein can slide back and forth between chamber 23 and 24. The reference numeral 10' is legs of the rack 25. The reference numeral 26 is a gas introducing pipe which leads a fluorine- or fluoride-containing gas into the fluoriding chamber23, 27 a temperature sensor, and 28 a nitriding gas introducing pipe. High-nickel based heat resistance alloy is desirable as material for the above-mentioned metallic muffle furnace 1 instead of stainless steel material.

This device is a continuous treatment system in which the inner temperature of a fluoriding chamber 23 is raised by the heating on nitriding in the nitriding chamber 24, nickel alloy articles are introduced into the fluoriding chamber 23 under that condition to be fluorided. After exhausting the gas in fluoriding chamber 23, the nickel alloy articles together with the metallic container are transferred to the nitriding chamber 24 by opening and shutting the barrier 22. And then, nitriding is carried out under that condition thereby conducting fluoriding and nitriding continuously.

The adoption of NF₃ as fluorine- or fluoride-containing gas is suitable in particular for the above-mentioned fluoriding. That is, NF₃ is a handy gaseous substance that has no reactivity at the ordinary temperature allowing operations and detoxication of exhaust gas to be easy.

### BRIEF DESCRIPTION OF THE DRAWINGS

Fig. 1 schematically shows a construction of a treatment furnace for carrying out nitriding according to the invention,
Fig. 2 schematically shows a construction of another furnace, for carrying out nitriding according to the invention,
Fig. 3 is an enlarged sectional view of a nitrided nickel alloy plate (inconel 600),
Fig. 4 is an enlarged sectional view of a nitrided nickel alloy plate (inconel 751), and
Fig. 5 is an enlarged sectional view of a nitrided nickel alloy plate (hastelloy C ).

The following modes for carrying out the invention illustrate the invention.

### Example 1

Three kinds of nickel alloy plates made of inconel 600 ( Ni:76, Cr:16, Fe:8 ), inconel 751 ( Ni:73, Cr:16, Ti:2.5 ), and hastelloy C ( Ni:56, Cr:16, Mo:7 ) were charged into a treatment furnace as shown in Fig. 1. After vacuum purging the inside of the furnace, it was heated to 550°C. Then, in that state, fluorine- or fluoride-containing gas ( NF₃ 10 Vol% + N₂ 90 Vol% ) was charged into the furnace to form an atmospheric pressure in it and the condition was maintained for 30 minutes. Then after exhausting the above-mentioned fluorine- or fluoride-containing gas out of the furnace, nitriding gas ( NH₃ 50 Vol% + N₂ 25 Vol% + H₂ 25 Vol% ) was introduced into the furnace and the inside of the furnace was heated to 570 °C. Nitriding treatment was carried out in this condition for 3 hours. Through this nitriding process, surface hardening layers B of a nitrided layer were formed on the surface of three kinds of Nickel alloy plates made of inconel 600, inconel 751, and hastelloy C respectively, and their thickness each was 15 µm, 12 µm, and 10 µm as shown in Fig. 3, Fig. 4, and Fig. 5. In these drawings, "A" shows base material of nickel alloy. Also surface hardness of those surface hardening layers B was Hv=800∼1,000 in each case.

### Example 2

As to three kinds of nickel alloy plates made of inconel 600, inconel 751, and hastelloy C respectively, fluoriding treatment was carried out in the same way as Example 1. Then nitriding treatment was carried out at the temperature of 620 °C for 3 hours to them while a mixed gas composed of NH₃ 50 Vol% + N₂ 50 Vol% was introduced into the furnaces as a nitriding gas. After nitriding them, fluoriding was carried out at the temperature of 620°C for 3 hours employing similar fluorine- or fluoride-containing gas mentioned to that of Example 1 and further nitriding treatment was carried out again at the temperature of 620°C for 3 hours employing the above-mentioned nitriding gas. In this way fluoriding and nitriding were put in practice two times each to three kinds of nickel alloy and thickness of the hard layers made of a nitrided layer formed on those surfaces was measured. As a result, the thickness of each hard layer of inconel 600, inconel 751, and hastelloy C was 25 µm, 20 µm, and 18 µm. It was found their surface hardness was the same as that of Example 1.

### Example 3

A mixed gas composed of F₂ 10 Vol% + N₂ 90 Vol% was employed as fluorine- or fluoride-containing gas. Except this difference, all the same fluoriding and nitriding treatments were carried out to three kinds of nickel alloy plates as Example 1. As a result, the same nitrided hard layers as Example 1 were formed on the surface of three kinds of plates after the treatments, and surface hardness was the same as that of Example 1.

As mentioned hereinbefore, the method of nitriding nickel alloy according to the invention comprises holding nickel alloy containing more than 25% nickel with heating in a fluorine- or fluoride- containing gas atmosphere at a temperature of 550-600°C to thereby eliminate organic and inorganic contaminants stuck to nickel alloy and at the same time causing an oxidised layer on the nickel alloy surface to be converted to a fluorinated layer, and then subjecting the alloy to the nitriding treatment. Since the oxidised layer on the nickel alloy surface is converted to a fluorinated layer in that manner, an existence of the fluorinated layer protects the nickel alloy surface. Therefore, even after a lapse of certain time from fluoriding to nitriding, the above-mentioned fluorinated layer protects the nickel alloy surface. As a result, no oxidized layer can be formed again on the nickel alloy surface. Since such a fluorinated layer can transmit "N" atoms, "N" atoms can penetrate uniformly into the nickel alloy surface layer to a certain depth at the time of nitriding. The resulting uniform penetration can lead to the formation of a close uniform nitriding layer in the depth only in the nickel alloy surface layer and the surface hardness is drastically improved without raising the base material stiffness of the nickel alloy.

## Claims

1. A method for nitriding nickel alloy comprising heating nickel alloy containing more than 25% nickel in a fluorine- or fluoride-containing gas atmosphere at temperature of 550-600°C to fluorinate the nickel alloy and heating the fluorinated nickel alloy in a nitriding atmosphere to form a nitrided layer in the surface layer of the nickel alloy.

2. A method for nitriding nickel alloy according to claim 1 in which the fluorine- or fluoride-containing gas atmosphere is composed of at least one of:
(a) a fluorine compound gas containing at least one component selected from the group; NF₃, BF₃, CF₄, HF, SF₆, C₂F₆, WF₆, CHF₃, and SiF₄;
(b) F₂ gas formed by cracking the above-mentioned fluorine compound gas (a); and
(c) pre-formed F₂ gas;
optionally together with an inert gas.

3. A method for nitriding nickel alloy according to any preceding claim in which the nitriding atmosphere is NH₃ gas, a mixture of NH₃ gas and RX gas, an inert gas mixture of an inert gas and NH₃ gas or NH₃ gas RX gas mixture, or a gas mixture formed by mixing H₂ gas with the inert gas mixture.

4. A method for nitriding nickel alloy according to any preceding claim in which the nickel alloy is heated in a nitriding atmosphere at a temperature between 500°C and 700°C.

## Patentansprüche

1. Verfahren zum Nitrieren einer Nickellegierung, umfassend Erhitzung einer Nickellegierung, die mehr als 25% Nickel enthält, in einer fluor- oder fluoridhaltigen Gasatmosphäre bei einer Temperatur von 550 - 600°C, um die Nickellegierung zu fluorieren und Erhitzen der fluorierten Nickellegierung in einer nitrierenden Atmosphäre, um eine nitrierte Schicht in der Oberflächenschicht der Nickellegierung zu bilden.

2. Verfahren zum Nitrieren einer Nickellegierung nach Anspruch 1, bei dem die fluor- oder fluoridhaltige Gasatmosphäre zusammengesetzt ist aus zumindest einem von:
(a) einem Fluorverbindungs-Gas enthalten mindestens eine Komponente ausgewählt aus der Gruppe: NF₃, BF₃, CF₄, HF, SF₆, C₂F₆, WF₆, CHF₃ und SiF₄;
(b) F₂-Gas gebildet durch Spaltung des vorgenannten Fluorverbindungs-Gases und
(c) vorgebildetes F₂-Gas;
wahlweise zusammen mit einem Inert-Gas.

3. Verfahren zum Nitrieren einer Nickellegierung nach einem der vorhergehenden Ansprüche, bei dem die nitrierende Atmosphäre NH₃-Gas, eine Mischung aus NH₃-Gas und RX-Gas, eine Inert-Gasmischung eines Inert-Gases und NH₃-Gas oder NH₃-Gas-RX-Gas-Mischung oder eine Gasmischung, die gebildet ist durch Mischung von H₂-Gas mit der Inert-Gasmischung, ist.

4. Verfahren zum Nitrieren einer Nickellegierung nach einem der vorhergehenden Ansprüche, bei dem die Nickellegierung in einer Nitrieratmosphäre auf eine Temperatur zwischen 500°C und 700°C erhitzt wird.

## Revendications

1. Procédé de nitruration d'un alliage de nickel comprenant le chauffage d'un alliage de nickel contenenant plus de 25% de nickel dans une atmosphère gazeuse contenant du fluor ou du fluorure à une température de 550-600°C pour fluorer l'alliage de nickel, et le chauffage de l'alliage de nickel fluoré dans une atmosphère nitrurante pour former une couche nitrurée sur la couche superficielle de l'alliage de nickel.

2. Procédé de nitruration d'un alliage de nickel selon la revendication 1, dans lequel l'atmosphère gazeuse contenant du fluor ou du fluorure est composée d'au moins l'un des gaz suivants:
(a) un gaz à composé fluoré contenant au moins un composant choisi parmi le groupe NF₃, BF₃, CF₄, HF, SF₆, C₂F₆, WF₆, CHF₃, et SiF₄;
(b) le gaz F₂ formé par craquage du gaz à composé fluoré (a) susmentionné; et
(c)le gaz F₂ préformé;
éventuellement conjointement avec un gaz inerte.

3. Procédé de nitruration d'un alliage de nickel selon l'une quelconque des revendications précédentes, dans lequel l'atmosphère nitrurante est le gaz NH₃, un mélange de gaz NH₃ et de gaz RX, un mélange gazeux inerte d'un gaz inerte et de gaz NH₃ ou d'un mélange de gaz NH₃ et de gaz RX, ou un mélange gazeux formé en mélangeant de gaz H₂ avec le mélange gazeux inertes

4. Procédé de nitruration d'un alliage de nickel selon l'une quelconque des revendications précédentes, dans lequel l'alliage de nickel est chauffé dans une atmosphère nitrurante à une température comprise entre 500°C et 700°C.
